

## UNITED STATES PATENT OFFICE

WILLIAM J. WRIGHTON AND EDGAR D. TILLYER, OF SOUTHBIDGE, MASSACHUSETTS,  
ASSIGNORS TO AMERICAN OPTICAL COMPANY, OF SOUTHBIDGE, MASSACHUSETTS,  
A VOLUNTARY ASSOCIATION OF MASSACHUSETTS

## PROCESS OF PLATING

No Drawing.

Application filed April 2, 1928. Serial No. 266,870.

This invention relates to improvements in metal articles and to an improved process of electro-plating the same, and has particular reference to an improved process for making such an article by plating it with the same material of which it is composed.

The principal object of the invention is to produce an improved homogeneous metallic article free from evidence of distortion due to 10 deforming the metal in producing the article.

Another object of the invention is to provide an improved process for plating a metal with its own material after the metal has been worked so as to eliminate the grain or other 15 evidences of distortion which has been produced by working the metal.

Another object of the invention is to provide an improved process for removing blemishes on the metal after it has been 20 worked by plating it with its own material.

Another object of the invention is to provide simple, efficient and economical means of plating an article after it has been worked to give it a finish that will eliminate working 25 blemishes.

Other objects and advantages of the invention will be apparent from the following description and it will be understood that changes may be made in the steps of the process 30 without departing from the spirit of the invention as expressed in the accompanying claims. We, therefore, do not wish to be limited to the exact matters described as the preferred forms and order of steps have been 25 given by way of illustration only.

It is well known that certain metals may be made and worked into finished articles but that the working will create a grain, a wave-like appearance or other blemishes or evidences of distortion in the finished article 40 due to the drawing, rolling and other operations through which the material has passed to produce the completed article. This causes the metal to look irregular and mars its appearance, particularly in articles where a high polish, luster and surface are required.

It is, therefore, the object of our invention to provide an improved process by which 50 these evidences of distortion may be removed and the article may be made of material

which hitherto could not be made due to these defects.

In the preferred form of the process we use the following procedure: If for example we wish to make an eyeglass frame, say of 55 nickel, we take a piece of nickel wire and draw it through the drawing rolls to the required size. We then roll it through the grooving rolls to roll in the lens receiving groove. This forms the eye wires of the 60 frame. We then roll the material for the bridge to desired proportions and bend the same for its connection to the rims and for the arch of the nose. We next provide end pieces for the temples which are preferably 65 pressed out in a die pressing machine. We then secure the ends of the bridge to the rims or eye wires and connect the two rims and then we fasten on the end pieces so that the rims or eye wires provide temple 70 connections. This produces an eyeglass frame completely made of nickel but on observation it will be found that the surface of the nickel 75 will show a grain, strain lines and other blemishes due to the drawing, rolling, pressing and other operations as described above in producing the article. These evidences of distortion are not only on the surface of the material but extend throughout the whole body of the material and cannot thus be removed by polishing, planing or other finishing operations, as could scratches or other surface blemishes which could be polished out or removed. We next polish the rough 80 frame which we have produced as described above until it has a smooth even surface and polish so it will receive the plating material. The article is then placed in a nickel electro-plating bath and is electro-plated with nickel, 85 which is the same material of which the rough article was made.

After the article is plated to a sufficient thickness it is removed from the bath and polished in the usual manner on buffing wheels and other polishing devices. The 90 plating will be smooth and uniform without the grain or evidences of distortion produced by the working being apparent, and surface blemishes and defects are also removed and a good looking commercial prod- 100

uct results. It will be noted that while the article is apparently a plated one, in reality it is one homogeneous article in which none of the evidences of distortion are visible.

In the foregoing description we have used nickel as the plating material and have produced a commercial eyeglass frame. It is clear that other materials which are capable of electro-plating can be used in the same way and that other articles than eyeglass frames can be produced.

From the foregoing description it will be seen that we have provided simple, efficient and economical means for producing our invention, carrying out our process to obtain the desired results.

Having described our invention, we claim:

1. The process of producing an article of manufacture from nickel whose properties are desired but which has a low elastic limit causing it to partially fracture and pit under ordinary shaping conditions, comprising shaping the nickel to the shape of the required article by stretching it beyond its elastic limit and thereafter filling the surface fractures and pits with nickel which has not been worked beyond its elastic limit.

2. An article of manufacture, the product of said process, comprising a nickel article, the main body of which has been stretched beyond its elastic limit and a supplemental coating of nickel which has not been stretched beyond its elastic limit, said coating of nickel filling in fractures and pits caused by stretching the main body beyond its elastic limit.

WILLIAM J. WRIGHTON.  
EDGAR D. TILLYER.